# EUROPEAN PATENT SPECIFICATION

(11) **EP 0 355 222 B1**
(45) Date of publication and mention of the grant of the patent: **27.10.1993**
(21) Application number: 88307697.8
(22) Date of filing: 19.08.1988
(51) Int. Cl.: D02J 13/00, D06B 3/04

(54) **Process of treating shrinkable fibers**
Verfahren zur Behandlung von schrumpffähigen Fasern
Procédé de traitement de fibres rétrécissables

(43) Date of publication of application: 28.02.1990
(73) Proprietor: E.I. DU PONT DE NEMOURS AND COMPANY, Wilmington Delaware 19898 (US)
(72) Inventor: Zatkulak, Tony Dominic, Midlothian Virginia 23112 (US); Rodini, David Joseph, Midlothian Virginia 23113 (US); Hodge, James Dwight, Midlothian Virginia 23113 (US)
(74) Representative: Jones, Alan John

(56) References cited:
- EP-A- 0 228 224
- GB-A- 1 193 725

## Description

The field of art to which this invention pertains is shrinkable materials and, more particularly, it is directed to processes for treating a tow of shrinkable fibers.

Specifically such invention is a process of treating a tow of aromatic polyamide fibers by moving the tow in folds through a chamber having a plug section which is operatively connected by a restricted opening to a treatment section and by heating the tow with steam in the treatment section.

Sufficient steam migrates into the plug section to cause shrinkage of the tow in this section. The cross-sectional area of the tow is substantially the same as the cross-sectional area of the entrance opening of the plug section as it enters such opening but it has a smaller cross-sectional area, due to shrinkage, as it leaves this section and moves through the restricted entrance opening of the treatment section. By making this opening smaller so that the cross-sectional area of the shrunken tow as it enters such restricted opening is substantially the same as the cross-sectional area of such opening, loss of steam through the entrance opening of the plug section is minimized.

More specifically, this invention is a process for dyeing a fiber structure of poly(meta-phenylene isophthalamide) fibers with a water-soluble dye by heating the amorphous, shrinkable fibers, as spun and prior to drying, with steam, in a specifically designed chamber, at a temperature from about 110°C. to about 140°C., and preferably at about 120°C., for a time sufficient to diffuse substantially all of the dye into the minute pores in the fibers, throughout the fiber structure.

An organic water-insoluble material, such as an ultraviolet light screener, may also be mixed with the water-soluble dye and padded onto the water-swollen fibers prior to heating.

While the dye is effectively diffused into the fiber structure at temperatures between 110°C. and 140°C., such structure must also be heated with steam at a sublimation temperature below the glass transition temperature of the fibers in order to sublime the screener into the pores of the fibers. The fibers are then, preferably, further heated with steam at about 165°C. for a time sufficient to collapse the pores in the fibers and lock the dye therein. At this temperature the fibers also will crystallize and the fiber structure is thereby stabilized against progressive laundry shrinkage.

### Description of the Related Art

Aromatic polyamide fibers are well known to the art. They have high tensile strength, are flame and heat resistant, possess good flex life, and have high melting points which make them particularly suited to be formed into fabrics usable as protective clothing, and for many other uses.

It further is known that while aromatic polyamide fibers possess many desired properties as manufactured they also require, for given uses, that various steps be taken to improve a property or properties of the fibers to meet a specific end use. As an example, various additives such as dyes, ultraviolet light screeners, flame retardants, antistatic agents or water repellents, may be incorporated into the fibers during basic manufacture or in subsequent processing steps to improve their performance levels.

GB-A-1 193 725 concerns continuous steaming of textile fibre material impregnated with dye liquor by feeding the material as partially superimposed folds into a convergent entry zone of an externally heated steaming passage to gradually compress the fibre mass, then through a restricted cross-sectional area in the presence of steam under pressure and then decompressing the steamed material in a divergent exit zone.

This invention is specifically directed to aromatic polyamide fibers of a poly(meta-phenylene isophthalamide) polymer, hereinafter referred to as "MPD-I fibers". Such fibers, which are described in greater detail in U. S. patent 3,287,324 to Sweeny, for example, possess many useful properties. It is well known to the art, however, that these fibers are difficult to dye.

Various techniques have evolved to solve this dyeing problem. One such solution is more fully described in copending EP-A-0 228 224 which application is incorporated herein by reference.

The invention of this copending application solves various problems found in the prior art by surprisingly finding that by heating as-spun, never-dried, water-swollen, or still moist to the touch, MPD-I fibers with steam, heated within certain temperature ranges, it is possible effectively to dye the fibers. Specifically, it has been found that such fibers may be dyed, using a water-soluble dye, by heating the fibers with steam heated at a temperature from about 110°C. to 140°C. for a time sufficient to diffuse the dye into the pores of the fibers.

It further has been found that after this diffusion step has taken place that such fibers may be subsequently heated, again with steam, at a temperature of about 165°C. to collapse the fibers and lock the dye in place. This latter step will also crystallize the fibers and stabilize them against progressive laundry shrinkage.

In practicing the invention just described, the treatment or dyeing of the fibers is accomplished by moving such fibers, in tow form, through a treatment chamber having one or more treatment sections. It has been found difficult to maintain the steam temperatures at the critical limits required, within these sections, since the steam tends to migrate toward the chamber openings. This problem is partially solved, as described in the above-mentioned copending EP-A-0 228 224, by supplying the tow to the chamber in folds. While this is an effective means of controlling the loss of steam, the problem still remains troublesome, particularly in the case of shrinkable tows because their cross-sections vary due to shrinkage as they move through the chamber. The instant invention not only solves this shrinkage problem but also provides an improved process for practicing the invention of copending EP-A-0 228 224.

Accordingly, this invention provides improved processes for treating aromatic polyamide fibers, using steam to dye a water-swollen fiber structure of poly(meta-phenylene isophthalamide) fibers with a water-soluble dye, before they are dried, or to add an organic water-insoluble material to the fibers, either mixed with the dye or alone, and to lock the dye and/or other impregnant into the pores of the fibers. This is accomplished by maintaining the steam within certain critical temperature ranges (e.g., 110°C. to 140°C.) in a specially designed chamber to diffuse the dye into the fiber pores and up to 165°C. to sublime the water-insoluble material into such pores. At this latter temperature the dye is also locked into the fibers, while stabilizing such fibers against progressive laundry shrinkage.

### Summary of the Invention

Briefly described, this invention is a process for treating synthetic fibers including the steps of:
moving a tow of shrinkable fibers in folds through a treatment section having an entrance opening and an exit opening smaller than the entrance opening and
heating the tow with steam in the treatment section.

In this process, the tow has a cross-sectional area substantially the same as the cross-sectional area of the entrance opening as it enters that opening whereby loss of steam through such opening is minimized and a smaller cross-sectional area as it leaves the section, due to shrinkage. This latter area is only slightly smaller, or substantially the same size as, the exit opening whereby loss of steam is minimized through this opening as well.

In a more specific embodiment, this invention is a process of treating a tow of shrinkable fibers which includes the steps of:
moving the tow in folds through a plug section operatively connected by a restricted opening to a treatment section, with the plug section having an entrance opening larger than the restricted opening of the treatment section, and
heating the tow with steam in the treatment section.

Sufficient steam migrates through the restricted opening from the treatment section to the plug section to cause shrinkage of the tow in the plug section. The tow has a cross-sectional area substantially the same as the cross-sectional area of the entrance opening of the plug section as it moves through this opening and has a smaller cross-sectional area as it leaves the plug section and moves through the entrance opening of the treatment section, due to shrinkage. The cross-sectional area of the shrunken tow as it enters the smaller entrance opening of the treatment section is substantially the same as the cross-sectional area of this opening and, along with the tow moving in folds in the plug section, this substanially prevents loss of steam through the entrance opening of the plug section.

Preferably the tow is an amorphous aromatic polyamide and, more specifically the aromatic polyamide is poly meta-phenylene isophthalamide). Such tow has a second order glass transition temperature in steam of above about 150°C.

The processes just described further may include the steps of padding a water-soluble dye onto the tow prior to the treatment section and heating the tow with steam in the treatment section at a temperature of from about 110°C. to 140°C. for a time sufficient to diffuse the dye into pores in the fibers of the tow. Still further steps may include moving the tow into a second treatment section and heating the tow with steam in this section at a temperature above its glass temperature from about 150°C. to 165°C. for a time sufficient to collapse the pores and lock the dye within the fibers and to crystallize such fibers and thereby stabilize the tow against progressive laundry shrinkage.

In still another embodiment, the process of this invention includes the steps of:
moving the tow through first and second treatment sections,
contacting the fibers of the tow prior to the first treatment section with an aqueous mixture containing a water-soluble dye and an organic water-insoluble material which sublimes in steam at a temperature below the glass transition temperature of the fibers,
heating the water-swollen fibers with steam in the first treatment section at a temperature from about 110°C. to 140°C. for a time sufficient to diffuse substantially all of the water-soluble dye into the pores of such fibers throughout the fiber structure,
heating the water-swollen fibers with steam at a sublimation temperature below the glass transition temperature of the fibers for a time sufficient to sublime the water-insoluble material into the pores of such fibers throughout the fiber structure, and thereafter
heating the water-swollen fibers with steam in the second treatment section at a temperature above the glass transition temperature of the fibers for a time sufficient to collapse the pores and irreversibly lock the dye within the fibers and to stabilize the fibers against progressive laundry shrinkage.

In this latter process, the fibers preferably are heated with steam at a sublimation temperature from about 110°C. to 150°C. The water-insoluble material may be an ultraviolet light screener and the water-insoluble material may be a disperse dye. Further the fibers may be heated with steam in the second treatment section at a temperature of about 165°C. to stabilize the fibers.

In more precise detail, this invention is a process of treating a tow of shrinkable material including the steps of:
moving the tow at a first speed through an entrance opening at one end of a funnel-shaped, fold-forming section having converging walls which define a discharge opening at the other end of the section, with the entrance opening being larger than the discharge opening;
moving the folded tow through a restricted entrance opening of a chamber defined by walls and having a plurality of sections including a plug section and first and second steam treatment sections, with the chamber being connected to the discharge opening of the fold-forming section and the chamber entrance opening being smaller than the entrance opening of fold-forming section, and the chamber further having a tow exit opening
wherein the dual action of the converging walls of the fold-forming section and the tow pushing through the restricted entrance opening of the chamber forms a plurality of folds in the tow,
wherein steam is introduced into the second steam treatment section, which is positioned between the entrance and exit openings of the chamber, whereby such steam flows,
in one direction into and through the second steam treatment section and into the first steam treatment section, and from there into the plug section and toward the entrance opening of the fold-forming section and
in the other direction into and through the second steam treatment section and toward the exit opening of the chamber,
engaging the folds of the tow as it is moved in the fold-forming section and through the entrance opening of the chamber with pins on an endless chain moving at a second speed slower than the first speed
moving the tow in folds through the plug section at the second speed and
wherein the plurality of folds of the tow are in substantial contact with the walls of chamber defining the plug section during a substantial portion of their movement through this section whereby to help substantially eliminate loss of steam through the entrance opening of the fold-forming section and
wherein the steam flowing into this plug section shrinks the tow so that it has a cross-sectional area smaller than that at which it entered this section
moving the tow in folds through a restricted entrance opening of the first treatment section, with such entrance opening being smaller than the entrance opening of the chamber
moving the tow through the first treatment section at the second speed and wherein the plurality of folds of the tow, as shrunken in the first plug section, are substantially in contact with the walls defining the first treatment section through much of their movement through this section whereby to further help prevent any loss of steam flowing though this section and through the plug section from escaping through the entrance opening of the fold-forming section.

In such process, preferably, the chain engages two tows, one on each side, and moves them at the second speed through the chamber and the entrance opening of the chamber is connected to discharge opening of the fold-forming section by a tapered surface. A tapered surface also preferably connects the plug section to the entrance opening of the treatment section.

Finally, in its broadest terms, this invention matches the shrinking profile of the tow with the profile of the chamber walls, during treatment of such tow in the chamber.

### Brief Description of the Drawing

Fig. 1 is a schematic view of an apparatus, including a treatment chamber suitable for practicing the process of this invention.

Figs. 2 and 2A are schematic views showing the chamber in greater detail.

Fig. 3 is a cross-sectional view taken along lines A-A of Fig. 1, which highlights a significant feature of this invention, in showing the substantial contact of the tow with the walls defining the restricted opening of the treatment section of the chamber as it is moved through that opening.

### Description of the Preferred Embodiments

This invention is an improved process for treating shrinkable materials, such as aromatic polyamide fibers.

More specifically,in the processes of this invention, a water-soluble material, and, if desired, a water-insoluble material are diffused or sublimed into a fiber structure of MPD-I amorphous synthetic fibers to improve their properties. During the diffusion and sublimation steps, the fibers are water-swollen or damp to the touch, with open pores. Steam controlled at critical temperatures in a chamber, is used to perfect the process.

Briefly, the fibers of this invention are prepared from aromatic polyamide polymers such as are disclosed in U. S. patent 3,063,966 to Kwolek, Morgan and Sorenson; 3,094,511 to Hill, Kwolek and Sweeny; and 3,287,324 to Sweeny, for example. These patents, and their teachings, are incorporated by reference into this application.

In preparing the basic water-swollen MPD-I fibers which are treated by the process of this invention, aromatic polyamides which have been prepared by procedures shown in the above-mentioned patents are combined with various solvents to form a spinning solution as shown, for example, in U. S. patent 3,063,966 and the fibers or filaments are formed by extruding the spinning solution through orifices in a spinneret. Such fibers may be dry-spun or wet-spun to form a water-swollen fiber structure. In either case, the fibers as spun are substantially amorphous.

The fibers whether dry-spun or wet-spun contain a substantial amount of solvent after having been solidified in a dry-spinning evaporation cell or coagulated in a wet-spinning precipitation bath. To remove the solvent such fibers are brought into contact with an aqueous extraction bath, as is known in the art. As a result the fibers become "water-swollen" with a water content of around 35% or more.

The above-described steps of forming amorphous water-swollen fibers of an aromatic polyamide polymer are known to the art and these fibers are all suitable for being further treated or processed in accordance with the process of this invention.

Specifically, in a preferred process, these water-swollen fibers, which have not been dried, are contacted with an aqueous solution containing a water-soluble material and heated with steam at a temperature from about 110°C. to 140°C. for a time sufficient to diffuse substantially all of the water-soluble material into the pores of the fibers throughout such fiber structure. The material diffused into the fibers preferably is a dye. It may also be a surfactant.

In another preferred embodiment, when the material is dyed, the water-swollen, dye-containing fibers are then further heated with steam at a temperature above the glass transition temperature of the fibers for a time sufficient to collapse the pores and irreversibly lock the dye within the fibers and to crystallize such fibers and stabilize them against progressive laundry shrinkage. Temperatures in the range from 150°C. to 165°C. will accomplish these objectives.

In still another embodiment, never-dried, amorphous MPD-I fibers of the type described are contacted with an aqueous mixture containing both a water-soluble material, such as a dye, and an organic water-insoluble material which sublimes in steam at a temperature below the glass transition temperature of the fibers. The water-swollen fibers are then heated with steam at a temperature from about 110°C. to 140°C. for a time sufficient to diffuse substantially all of the water-soluble dye into the pores of such fibers and at a sublimation temperature below the glass transition temperature of the fibers to sublime the water-insoluble material into the open pores of such fibers. After the diffusion and sublimation steps have been completed, the fibers may be further heated with steam at a temperature above the glass transition temperature of the fibers for a time sufficient to collapse the pores and irreversibly lock the material within the fibers and to stabilize the fibers against progressive laundry shrinkage.

The term "fiber", as used herein, includes both staple fibers and continuous filaments. The continuous filaments may be in the form of a tow containing a large number of filaments or in the form of a yarn.

Referring specifically to Figure 1 of the drawing, a fiber structure of never-dried, shrinkable fibers, as spun, in large bundles called tow, as indicated by the reference numeral 1, is supplied from a supply source 2 and passed over guide rolls 3 to nip rolls 4 and 4′.

An aqueous bath 5 of constant level is maintained at the entrance to the nip rolls. The tow 1 of moist to the touch fibers is brought into contact with the bath 5 which contains the material (e.g., a water-soluble dye, or surfactant, or ultraviolet light screener, for example) to be diffused or sublimed into the fibrous tow. The pick-up of material on the never-dried tow may be adjusted by suitably controlling the speed of the tow and the pressure applied between the nip rolls.

The tow 1 coated with the desired amount of material is then moved by feed rolls 6 into a treatment chamber 7, which is suitably an elongated tube having two or more treatment sections to which steam under appropriate pressure can be supplied, as will be explained in greater detail.

The tow is heated in these treatment sections at the required critical temperatures to diffuse the water-soluble material and to sublime the insoluble material into the fibers, after which such fibers may be further heated to stabilize the fiber structure against progressive laundry shrinkage.

The processed tow is then moved out of the chamber 7 and onto a conveyor 8, and then through squeeze rolls 9 to help remove water from the treated tow. The tow is then fed by feed rolls 10 into a dryer 11, which includes upper and lower conveyors 12 and 13 which move the tow at a speed which is adapted to form folds in the tow in the dryer. Such conveyors move the tow through the dryer 11 for a time sufficient to remove substantially all of the water from the tow. The dried and processed tow is then moved over transfer rolls 14 and into a storage container 15.

The treatment process will now be described in detail.

The tow 1 carrying the dye or other treatment material from the bath 5 is fed by feed rolls 6 at a first speed through an entrance opening 17 at one end of a funnel-shaped, fold-forming section 18 having converging walls 19 which define a discharge opening 20 at the other end of the section.

The tow is then moved through a restricted entrance opening 21 of the treatment chamber 7 defined by walls 22 and having a plurality of sections including a plug section 23 and first and second steam treatment sections 24 and 25. The chamber 7 is connected, preferably by a sharply tapered surface 22′ to the discharge opening 20 of the fold-forming section 18 and the chamber entrance opening 21 is smaller than the entrance opening 17 of the fold-forming section 18. The dual action of the converging walls of the fold-forming section 18 and the tow 1 pushing through the restricted entrance opening 21 of the chamber 7 forms a plurality of folds in the tow. The chamber 7 further has a tow exit opening 26.

Steam in introduced into the second steam treatment section 25 which is positioned between the entrance and exit openings 21, 26 of the chamber 7. The steam flows in one direction into the second steam treatment section 25, then through this section and into the first steam treatment section 24, and from there into the plug section 23 and toward the entrance opening 17 of the fold-forming section 18 and in the other direction into and through the second steam treatment section 25 and toward the exit opening 26 of the chamber 7.

As best seen in Figure 3, the folds of the tow 1 are engaged by pins 27 on an endless chain 28 as the tow is moving in fold-forming section 18 and through the entrance opening 21 of the chamber 7. The chain 28 moves at a second speed slower than the first speed at which the tow is fed into the fold-forming section 18, by feed rolls 6.

The tow is moved in folds through the plug section 23 at this second speed. In this section 23 the plurality of folds of the tow are in substantial contact with the walls of chamber 7 during a substantial portion of their movement through such section whereby to help substantially eliminate loss of steam through the entrance opening 17 of the fold-forming section 18. The steam flowing into this plug section 18 shrinks the tow so that it has a cross-sectional area smaller than that at which it entered the section. The tow is then moved from the plug section 23 and a restricted entrance opening 29 of the first treatment section 24. The restricted entrance opening 29 is smaller than the restricted entrance opening 21 of the chamber 7.

The tow is moved through the first treatment section 24 at the second speed and the plurality of folds of the tow, as shrunken in the plug section 23, are substantially in contact with the walls defining the first treatment section 24 through much of their movement through such section whereby to further help prevent any loss of steam flowing through this section 24 and through the plug section 23 from escaping through the entrance opening 17 of the fold-forming section 18. This invention provides better control of steam temperatures in the critical treatment sections of the chamber.

The substantial contact of the folded tow with the walls of the chamber 7, pushing through the restricted entrance opening 21 of the plug section 23 and hence through the restricted opening 29 of the first treatment section 24, along the contact of the folds with the walls 22 in these sections, substantially prevents escape of steam through the entrance opening of the chamber.

In this same connection, it frequently is desirable to wash the treated fibers in a wash section 30 of the chamber 7 prior to discharge of the tow from such chamber. The wash water along with the folded tow, further combine to substantially prevent loss of steam through the exit opening 26 of the chamber, as well.

By controlling loss of steam through the chamber openings, it is possible to maintain better control of the critical temperatures required in the first and second treatment sections, to effectively treat the fibers, as previously described.

The treatment of the tow in the manner just described provides MPD-I fibers having the improved properties sought in the treatment.

The following example will further illustrate this invention.

### Example

### A. Preparation of Never-Dried Filaments of Poly(metaphenylene isophthalamide) (MPD-I).

Filaments of MPD-I having an inherent viscosity of 1.5 were dry spun from a filtered solution containing 19% MPD-I, 70% dimethylacetamide (DMac), 9% calcium chloride, and 2% water. On leaving the drying tower the as-spun filaments were given a preliminary wash with water so that they contained about 60% DMac, 15% calcium chloride, and 100-150% water, based on the weight of dry polymer. The filaments were washed and drawn 4X at 90°C. in a counter-current extraction-draw process in which the calcium chloride determined as chloride content and DMac content were reduced to about 0.1% and 0.5%, respectively. The wet filaments were gathered together to form a tow, a conventional antistatic finish was applied to the tow, and the tow was crimped in a stuffer box crimper at a temperature of about 80°C. in the presence of steam. The tow was then collected, still moist to the touch, in a plastic-lined cardboard box. The individual filaments had a linear density of about 1.55 decitex (dtex) (1.7 dpf). The linear density of the never-dried filaments here and elsewhere herein is based on the weight of dry filaments.

### B. Dyeing and Shrinkage Stabilization of Tows of Never-Dried MPD-I Filaments in a Steam Chamber.

Two 120-kilotex (1,000,000 denier) tows of never-dried MPD-I filaments, prepared as described in Part (A) above, were creeled through the guides of a continuous tow dyeing apparatus equipped for high shrinkage tow. The tows were first fed between nip rolls at a rate of 14 m/min. wherein an aqueous dye solution was padded onto the tow so that the individual filaments in the tow were coated with the solution. The solution contained 40 g/l of C.I. (Colour Index) No. Basic Yellow 28 dye (a water-soluble dye), and 6 g/l of C.I. No. Basic Red 15 (a water-soluble dye), and 6 g/l cellulosic thickner, and 58 g/l of anionic surfactant, adjusted to a pH of 7 (adding acetic acid or caustic soda as needed until the desired pH was obtained). The pick-up of the dye solution on the tow as 30 weight %.

After the tows were padded with the dye solution, they were then passed through the entrance funnel of a chamber, such as that shown in Figure 2, the rectangular discharge end of the funnel having a width of 95 mm and a depth of 115 mm. Within the funnel the tows were turned and then gathered into folds as they were picked up by a chain moving at 1 m/min., one tow on each side of the chain. The tows, carried by the chain, were then passed into the entrance opening of a plug section of the chamber, which had a rectangular cross section 90 mm in width and 110 mm in depth, the discharge opening of the funnel and the entrance opening of the plug section being gently tapered into one another to avoid a stair step transition. The plug section was 3 m in length, and from it the tows were carried by the chain into a first treatment section, also 3 m in length, which had a rectangular cross section 88 mm in width and 107 mm in depth, the transition from the plug section to the first treatment section being gently tapered to avoid a stair-step transition. From the first treatment section the tows were then carried by the chain into a second treatment section 6 m in length wherein the tows of filaments coated with the solution were exposed to steam at a pressure of 609 kPa (six bars) and a temperature of 165°C. the steam being introduced into the chamber through holes in the walls of the chamber. The steam flowed from the second steam section back into the first treatment section and then into the plug section at progressively lower pressures and temperatures in the direction of the entrance funnel, the folds of the tow effectively sealing the entrance to the plug section so that substantially no steam flowed back into the entrance funnel. Within a zone beginning at about the end of the plug section and extending well into the first treatment section the filaments in the tows coated with the solution were exposed to steam at a temperature of about 120°C. for a contact time of about two minutes. The temperature of the tows at the end of the first treatment section, going into the second steam treatment section, was about 165°C. and remained at about 165°C. throughout the second treatment section. Upon leaving the treatment sections the tows were passed into a final wash section, wherein they were washed with water. The water and the wet tows acted together to condense the steam flowing from the second treatment section and formed an effective seal to prevent any steam from flowing from the exit end of the chamber.

After the tows were washed, they were fed into a forced air dryer, wherein their moisture level was reduced to 7% moisture. Finish was not added to the tow. The tows were dyed to a bright shade of orange. The shrinkage of the tows was measured and determined to be 0.9%.

In other experiments with similar tows using apparatus having a steam chamber of constant area, it was found to be difficult to maintain the steam at a pressure higher than about 203 kPa (two bars). The shrinkage of the tow when heated with steam at a pressure of only 203 kPa was 7%.

## Claims

1. A process for treating a tow (1) of shrinkable poly (meta-phenylene isophthalamide) fibre with steam wherein the tow is passed in folds through an entrance opening (17) to and through an elongated treatment chamber (7) to which steam under appropriate pressure is supplied and out of an exit opening (20) of the chamber (7) and during which passage, the tow shrinks, characterised by minimising the loss of steam through the entrance and exit openings by restricting the entrance opening to a cross-sectional area substantially the same as that of the folded tow entering the chamber (7) and restricting the exit opening to a cross-sectional area smaller than the entrance opening and substantially the same as that of the folded tow leaving the chamber (7).

2. A process according to claim 1 wherein the folded tow is moved through the chamber by engagement with an endless chain (28).

3. A process according to claim 1 wherein a water-soluble dye is padded onto the tow prior to passage through the treatment chamber (7) and the tow is treated in such chamber with steam at from 110°C for a time sufficient to diffuse the dye into pores of the fibres of the tow.

4. A process according to claim 3 wherein the tow leaving the treatment chamber (7) is heated in steam at a temperature above its glass transition temperature, at about 150°C to 165°C for a time sufficient to collapse the pores to lock the dye within the fibres and to stabilise the tow against shrinkage.

5. The method of any one of claims 1 to 4 including the further steps of:
moving the tow through first (24) and second (25) treatment sections,
contacting the fibres of the tow prior to the first treatment section with an aqueous mixture containing a water-soluble dye and an organic water-insoluble material which sublimes in steam at a temperature below the glass transition temperature of the fibres,
heating the fibres with steam in the first treatment section (24) at a temperature from about 110°C to 140°C for a time sufficient to diffuse substantially all of the water-soluble dye into the pores of such fibres throughout the fibre structure,
heating the water-swollen fibres with steam at a sublimation temperature below the glass transition temperature of the fibres for a time sufficient to sublime the water-insoluble material into the pores of such fibres throughout the fibre structure, and thereafter
heating the water-swollen fibres with steam in the second treatment section (25) at a temperature above the glass transition temperature of the fibres for a time sufficient to collapse the pores and irreversibly lock the dye within the fibres and to stabilise the fibres against progressive laundry shrinkage.

6. The process of claim 8 wherein the fibres are heated with steam in the first treatment section (24) at a sublimation temperature of from about 110°C to 150°C.

7. The process of claim 5 or claim 6 wherein the water-insoluble material is an ultraviolet light screener or a disperse dye.

8. The process of any one of claims 5 to 7 wherein the fibres are heated with steam in the second treatment section (25) at a temperature of about 165°C.

9. A process of treating a tow of shrinkable material which comprises the steps of:
moving the tow (1) at a first speed through an entrance opening (17) at one end of a funnel-shaped, fold-forming section (18) having converging walls (19) which define a discharge opening at the other end of the section, said entrance opening (17) being larger than the discharge opening (20);
moving the folded tow through a restricted entrance opening of a chamber defined by walls and having a plurality of sections including a plug section (23) and first (24) and second (25) steam treatment sections, said chamber being connected to the discharge opening of the fold-forming section (18) and said chamber entrance opening being smaller than the entrance opening (17) of the fold-forming section (18), said chamber further having a tow exit opening
wherein the dual action of the converging walls of the fold-forming section and the tow pushing through said restricted entrance opening of the chamber forms a plurality of folds in the tow,
wherein steam is introduced into the second steam treatment section (25), which is positioned between the entrance and exit openings of the chamber, whereby such steam flows,
in one direction into the second steam treatment section (25), then through this section and into the first steam treatment section (24), and from there into the plug section (23) and toward the entrance opening (17) of the fold-forming section and
in the other direction into and through the second steam treatment section (25) and toward the exit opening (26) of the chamber,
engaging the folds of the tow as it is moved in the fold-forming section and through the entrance opening (17) of the chamber with pins (27) on an endless chain (28) moving at a second speed slower than the first speed
moving the tow in folds through the plug section (23) at said second speed and
wherein the plurality of folds of the tow are in substantial contact with the walls of chamber defining the plug section (23) ring a substantial portion of their movement through this section whereby to help substantially eliminate loss of steam through the entrance opening of the fold-forming section (18) and
wherein the steam flowing into this plug section shrinks the tow so that it has a cross-sectional area smaller than that at which it entered this section
moving the tow in folds through a restricted entrance opening of the first treatment section, said entrance opening being smaller than the restricted entrance opening of the chamber
moving the tow through the first treatment section (24) at said second speed and wherein the plurality of folds of the tow, as shrunken in the plug section (23), are substantially in contact with the walls defining the first treatment section (24) through much of their movement through this section whereby to help further prevent any loss of steam flowing through this section and through the plug section (23) from escaping through the entrance opening of the fold-forming section.

10. The process of claim 9 in which the chain engages two tows, one on each side, and moves them at said second speed through the chamber.

11. The process of claim 9 or claim 10 in which the restricted entrance opening of the chamber is connected to discharge opening of the fold-forming section (18) by a tapered surface (19).

12. The process of claim 9, 10 or 11 in which the restricted entrance opening of the first treatment section (24) is connected to the plug section (23) by a tapered surface.

13. An apparatus for treating a tow of shrinkable material which comprises:
means for moving the tow (1) at a first speed through an entrance opening (17) at one end of a funnel-shaped, fold-forming section (18), said section having converging walls (19) which define a discharge opening at the other end of the section and said entrance opening (17) being larger than the discharge opening (20);
means for moving the folded tow through a restricted entrance opening of a chamber defined by walls and having a plurality of sections including a plug section (23) and first (24) and second (25) steam treatment sections, said chamber being connected to the discharge opening of the fold-forming section (18) and said chamber entrance opening being smaller than the entrance opening (17) of the fold-forming section (18), said chamber further having a tow exit opening;
means for introducing steam into the second steam treatment section (25), which is positioned between the entrance and exit openings of the chamber, so that such steam flows in one direction into the second steam treatment section (25), thereafter through this section and into the first steam treatment section (24), and from there into the plug section (23) and toward the entrance opening (17) of the fold-forming section and in the other direction into and through the second steam treatment section (25) and toward the exit opening (26) of the chamber;
means for engaging the folds of the tow as it is moved in the fold-forming section and through the entrance opening (17) of the chamber with pins (27) on an endless chain (28) moving at a second speed slower than the first speed;
means for moving the tow in folds through the plug section (23) at said second speed so that the plurality of folds of the tow are in substantial contact with the walls of chamber defining the plug section (23) during a substantial portion of their movement through this section, and so that the steam flowing into this plug section shrinks the tow so that it has a cross-sectional area smaller than that at which it entered this section;
means for moving the tow in folds through a restricted entrance opening of the first treatment section, said entrance opening being smaller than the restricted entrance opening of the chamber; and
means for moving the tow through the first treatment section (24) at said second speed so that the plurality of folds of the tow, as shrunken in the plug section (23), are substantially in contact with the walls defining the first treatment section (24) through much of their movement through this section.

## Patentansprüche

1. Verfahren zum Behandeln eines Kabels (1) aus schrumpffähiger (Meta-phenylenisophthalamid)-Faser mit Dampf, bei dem das Kabel in Falten durch eine Eintrittsöffnung (17) und durch eine längliche Behandlungskammer (7) geführt wird, welcher Dampf unter einem geeigneten Druck zugeführt wird, und das aus einer Austrittsöffnung (20) der Kammer (7) austritt, wobei während des Durchgangs das Kabel schrumpft, dadurch **gekennzeichnet,** daß zur Minimierung des Dampfverlustes durch die Eintritts- und Austrittsöffnung die Eintrittsöffnung auf eine Querschnittsfläche begrenzt ist, welche im wesentlichen gleichgroß wie jene des in Falten gelegten Kabels ist, welches in die Kammer (7) eintritt und die Austrittsöffnung auf eine Querschnittsfläche begrenzt wird, welche kleiner als jene der Eintrittsöffnung ist und die im wesentlichen gleich wie jene des in Falten gelegten Kabels ist, welches die Kammer (7) verläßt.

2. Verfahren nach Anspruch 1, bei dem das in Falten gelegte Kabel durch die Kammer in Zusammenarbeiten mit einer endlosen Kette (28) bewegt wird.

3. Verfahren nach Anspruch 1, bei dem ein wasserlöslicher Farbstoff mittels eines Kissens auf das Kabel vor dem Durchgang durch die Behandlungskammer (7) aufgetragen wird und das Kabel in dieser Kammer mit Dampf, ausgehend von etwa 110°C, eine derart ausreichende Zeit behandelt wird, daß der Farbstoff in die Poren der Fasern des Kabels diffundiert.

4. Verfahren nach Anspruch 3, bei dem das die Behandlungskammer (7) verlassende Kabel im Dampf auf eine Temperatur oberhalb der Glasübergangstemperatur, auf etwa 150°C bis 165°C eine derart ausreichende Zeit erwärmt wird, daß die Poren zusammensinken, um den Farbstoff in den Fasern festzulegen und das Kabel gegenüber einem Schrumpfen zu stabilisieren.

5. Verfahren nach einem der Ansprüche 1 bis 4, welches ferner die folgenden Schritte umfaßt:
Bewegen des Kabels durch einen ersten (24) und einen zweiten (25) Behandlungsteil,
Kontaktieren der Fasern des Kabels vor dem ersten Behandlungsteil mit einem wäßrigen Gemisch, welches einen wasserlöslichen Farbstoff und ein organisches, wasserunlösliches Material enthält, welches im Dampf bei einer Temperatur unterhalb der Glasübergangstemperatur der Fasern sublimiert,
Erwärmen der Fasern mit Dampf in dem ersten Behandlungsteil (24) bei einer Temperatur von etwa 110°C bis etwa 140°C eine so ausreichend lange Zeit, daß im wesentlichen der gesamte wasserlösliche Farbstoff in die Poren dieser Fasern durch die gesamte Faserstruktur hindurch diffundiert,
Erwärmen der mittels Wasser geschwollenen Fasern mit Dampf bei einer Sublimationstemperatur unterhalb der Glasübergangstemperatur der Fasern eine derart ausreichend lange Zeit, daß das wasserunlösliche Material in den Poren dieser Fasern durch die Faserstruktur hindurch sublimieren kann, und
anschließendes Erwärmen der mittels Wasser geschwollenen Fasern mit Dampf in einem zweiten Behandlungsteil (25) bei einer Temperatur oberhalb der Glasübergangstemperatur der Fasern eine so ausreichend lange Zeit, daß die Poren einfallen und der Farbstoff in den Fasern irreversibel festgehalten ist und daß die Fasern gegenüber einem progressiven Schrumpfen beim Waschen stabilisiert werden.

6. Verfahren nach Anspruch 8, bei dem die Fasern mit Dampf im ersten Behandlungsteil (24) bei einer Sublimationstemperatur von etwa 110°C bis 150°C erwärmt werden.

7. Verfahren nach Anspruch 5 oder Anspruch 6, bei dem das wasserunlösliche Material eine Ultraviolettlicht-Siebdruckeinrichtung oder ein dispergierter Farbstoff ist.

8. Verfahren nach einem der Ansprüche 5 bis 7, bei dem die Fasern mit Dampf im zweiten Behandlungsteil (25) bei einer Temperatur von etwa 165°C erwärmt werden.

9. Verfahren zum Behandeln eines Kabels aus schrumpffähigem Material, welches die folgenden Schritte aufweist:
Bewegen des Kabels (1) mit einer ersten Geschwindigkeit durch eine Eintrittsöffnung (17) an einem Ende eines trichterförmigen, faltenbildenden Teils (18), welches konvergierende Wände (19) hat, welche eine Ausgabeöffnung am anderen Ende des Teils bilden, wobei die Eintrittsöffnung (17) größer als die Ausgabeöffnung (20) ist;
Bewegen des in Falten gelegten Kabels durch eine begrenzte Eintrittsöffnung einer Kammer, welche von Wänden gebildet wird und eine Mehrzahl von Teilen hat, welche ein Stopfenteil (23) und ein erstes (24) und ein zweites (25) Dampfbehandlungsteil umfassen, wobei die Kammer mit der Ausgabeöffnung des faltenbildenden Teils (18) verbunden ist und die Kammereintrittsöffnung kleiner als die Eintrittsöffnung (19) des faltenbildenden Teils (18) ist und die Kammer ferner eine Kabelaustrittsöffnung hat,
wobei die Doppelwirkung der konvergierenden Wände des faltenbildenden Teils und des Durchdrückens des Kabels durch die begrenzte Eintrittsöffnung der Kammer zu der Bildung einer Mehrzahl von Falten im Kabel führt,
wobei Dampf in das zweite Dampfbehandlungsteil (25) eingeleitet wird, welches zwischen der Eintritts- und der Austrittsöffnung der Kammer angeordnet ist, durch welche dieser Dampf strömt,
in einer Richtung in das zweite Dampfbehandlungsteil (25) dann durch dieses Teil und in das erste Dampfbehandlungsteil (24) und von dort in das Stopfenteil (23) und zu der Eintrittsöffnung (17) des faltenbildenden Teils, und
in der anderen Richtung in und durch das zweite Dampfbehandlungsteil (25) und zu der Austrittsöffnung (26) der Kammer,
Zusammenwirken der Falten des Kabels bei der Bewegung in dem faltenbildenden Teil und durch die Eintrittsöffnung (17) der Kammer mit Stiften (27) auf einer endlosen Kette (28), welche sich mit einer zweiten, langsameren Geschwindigkeit als die erste Geschwindigkeit bewegt,
Bewegen des Kabels in Falten gelegt durch das Stopfenteil (23) mit der zweiten Geschwindigkeit, und
wobei die Mehrzahl von Falten des Kabels im wesentlichen in Kontakt mit den Wänden der Kammer ist, welche das Stopfenteil (23) bilden, und zwar während einem beträchtlichen Teil der Bewegung durch dieses Teil, wodurch in unterstützender Weise ein Dampfverlust durch die Eintrittsöffnung des faltenbildenden Teils (18) verhindert wird, und
wobei der Dampf, welcher in das Stopfenteil strömt, das Kabel derart schrumpft, daß es eine Querschnittsfläche hat, welche kleiner als jene ist, an der es in dieses Teil eintritt,
Bewegen des in Falten gelegten Kabels durch eine begrenzte Eintrittsöffnung des ersten Behandlungsteils, wobei die Eintrittsöffnung kleiner als die begrenzte Eintrittsöffnung der Kammer ist,
Bewegen des Kabels durch das erste Behandlungsteil (24) mit der zweiten Geschwindigkeit, wobei die Mehrzahl von Falten des Kabels geschrumpft in dem Stopfenteil (23) im wesentlichen in Kontakt mit den Wänden ist, welche das erste Behandlungsteil (24) bilden, und zwar über den Großteil der Bewegung durch dieses Teil hinweg, wobei in unterstützender Weise ferner ein Dampfverlust über dieses Teil und über das Stopfenteil (23) verhindert wird und ein Entweichen durch die Eintrittsöffnung des faltenbildenden Teils verhindert wird.

10. Verfahren nach Anspruch 9, bei dem die Kette mit zwei Kabeln auf jeder Seite zusammenarbeitet und diese mit der zweiten Geschwindigkeit durch die Kammer bewegt.

11. Verfahren nach Anspruch 9 oder Anspruch 10, bei dem die begrenzte Eintrittsöffnung der Kammer mit einer Ausgabeöffnung des faltenbildenden Teils (18) über eine konisch ausgebildete Fläche (19) verbunden ist.

12. Verfahren nach Anspruch 9, 10 oder 11, bei dem die begrenzte Eintrittsöffnung des ersten Behandlungsteils (24) mit dem Stopfenteil (23) über eine konische Fläche verbunden ist.

13. Vorrichtung zum Behandeln eines Kabels aus schrumpffähigem Material, welche folgendes aufweist:
eine Einrichtung zum Bewegen des Kabels (1) mit einer ersten Geschwindigkeit durch eine Eintrittsöffnung (17) an einem Ende eines trichterförmigen, faltenbildenden Teils (18), wobei dieses Teil konvergierende Wände (19) hat, welche eine Ausgabeöffnung am anderen Ende des Teils bilden, und wobei die Eintrittsöffnung (17) größer als die Ausgabeöffnung (20) ist;
eine Einrichtung zum Bewegen des in Falten gelegten Kabels durch eine begrenzte Eintrittsöffnung einer Kammer, welche von Wänden begrenzt wird, und die eine Mehrzahl von Teilen hat, welche ein Stopfenteil (23) und ein erstes (24) und ein zweites (25) Dampfbehandlungsteil umfassen, wobei die Kammer mit der Ausgabeöffnung des faltenbildenden Teils (18) verbunden ist und die Kammereintrittsöffnung kleiner als die Eintrittsöffnung (17) des faltenbildenden Teils (18) ist, und wobei die Kammer ferner eine Kabelaustrittsöffnung hat;
eine Einrichtung zum Einleiten von Dampf in das zweite Dampfbehandlungsteil (25), welches zwischen der Eintritts- und und der Austrittsöffnung der Kammer angeordnet ist, so daß der Dampf in eine Richtung in das zweite Dampfbehandlungsteil (25) strömt, anschließend durch dieses Teil und in das erste Dampfbehandlungsteil (24) strömt, und von dort in das Stopfenteil (23) und zu der Eintrittsöffnung (17) des faltenbildenden Teils strömt und in der anderen Richtung in und durch das zweite Dampfbehandlungsteil (25) und zu der Austrittsöffnung (26) der Kammer strömt;
eine Einrichtung zum Zusammenarbeiten mit den Falten des Kabels, wenn dieses in dem faltenbildenden Teil und durch die Eintrittsöffnung (17) der Kammer bewegt wird, wobei die Falten mit Stiften (27) einer endlosen Kette (28) zusammenarbeiten, welche sich mit einer zweiten Geschwindigkeit bewegt, welche kleiner als die erste Geschwindigkeit ist;
eine Einrichtung zum Bewegen des in Falten gelegten Kabels durch das Stopfenteil (23) mit dieser zweiten Geschwindigkeit, so daß die Mehrzahl von Falten des Kabels im wesentlichen in Kontakt mit den Wänden der das Stopfenteil (23) bildenden Kammer während eines beträchtlichen Teils ihrer Bewegung durch dieses Teil ist, und so daß der in das Stopfenteil strömende Dampf das Kabel schrumpft, so daß seine Querschnittsfläche kleiner als jene ist, mit der es in dieses Teil eintritt;
eine Einrichtung zum Bewegen des in Falten gelegten Kabels durch eine begrenzte Eintrittsöffnung des ersten Behandlungsteils, wobei die Eintrittsöffnung kleiner als die begrenzte Eintrittsöffnung der Kammer ist; und
eine Einrichtung zum Bewegen des Kabels durch das erste Behandlungsteil (24) mit dieser zweiten Geschwindigkeit, so daß die Mehrzahl von Falten des Kabels, welche im Stopfenteil (23) geschrumpft wurden, im wesentlichen in Kontakt mit den Wänden ist, welche das erste Behandlungsteil (24) begrenzen, und zwar über den Großteil der Bewegung durch dieses Teil.

## Revendications

1. Procédé permettant de traiter un fil (1) de fibre de poly(métaphénylène isophtalamide) rétrécissable avec de la vapeur, dans lequel on fait passer le fil replié (formant des plis) par une ouverture d'entrée (17), jusqu'à une chambre de traitement (7), qu'il traverse, et dans laquelle on introduit de la vapeur sous une pression appropriée, et on le fait passer par une ouverture de sortie (20) de la chambre (7), passage au cours duquel le fil se rétrécit, caractérisé en ce que l'on minimise la perte de vapeur par les ouvertures d'entrée et de sortie en limitant l'ouverture d'entrée à une superficie de section pratiquement identique à celle du fil replié entrant dans la chambre (7) et en limitant l'ouverture de sortie à une superficie de section inférieure à celle de l'ouverture d'entrée et pratiquement identique à celle du fil replié sortant de la chambre (7).

2. Procédé selon la revendication 1 dans lequel le fil est déplacé dans la chambre par engagement avec une chaîne à chenille (28).

3. Procédé selon la revendication 1, dans lequel on enduit le fil d'un colorant hydrosoluble avant le passage dans la chambre de traitement (7), puis on traite le fil dans cette chambre avec de la vapeur à partir de 110°C, suffisamment longtemps pour diffuser le colorant dans les pores des fibres du fil.

4. Procédé selon la revendication 3 dans lequel on chauffe le fil sortant de la chambre de traitement (7) dans de la vapeur à une température supérieure à sa température de transition vitreuse, d'environ 150°C à 165°C, suffisamment longtemps pour fermer les pores afin de retenir le colorant à l'intérieur des fibres et de stabiliser le fil contre le rétrécissement.

5. Procédé selon l'une quelconque des revendications 1 à 4 comprenant en outre les étapes:
de passage du fil dans des première (24) et seconde (25) sections de traitement,
de mise en contact des fibres du fil, avant la première section de traitement, avec un mélange aqueux contenant un colorant hydrosoluble et une matière organique insoluble dans l'eau, qui se sublime dans la vapeur à une température inférieure à la température de transition vitreuse des fibres,
de chauffage des fibres à la vapeur dans la première section de traitement (24), à une température d'environ 110°C à 140°C, suffisamment longtemps pour diffuser pratiquement tout le colorant hydrosoluble dans les pores de ces fibres, à travers la totalité de la structure des fibres,
de chauffage à la vapeur des fibres gonflées par l'eau, à une température de sublimation inférieure à la température de transition vitreuse des fibres, suffisamment longtemps pour sublimer la matière insoluble dans l'eau en la faisant pénétrer dans les pores de ces fibres, à travers la totalité de la structure des fibres, puis
de chauffage à la vapeur des fibres gonflées par l'eau, dans la seconde section de traitement (25), à une température supérieure à la température de transition vitreuse des fibres, suffisamment longtemps pour fermer les pores et retenir de façon irréversible le colorant à l'intérieur des fibres et stabiliser les fibres contre le rétrécissement progressif lors des lessives.

6. Procédé selon la revendication 8, dans lequel on chauffe les fibres à la vapeur dans la première section de traitement (24) à une température de sublimation d'environ 110°C à 150°C.

7. Procédé selon la revendication 5 ou la revendication 6, dans lequel la matière insoluble dans l'eau est un filtre pour la lumière ultraviolette ou un colorant de dispersion.

8. Procédé selon l'une quelconque des revendications 5 à 7, dans lequel on chauffe les fibres à la vapeur dans la seconde section de traitement (25) à une température d'environ 165°C.

9. Procédé permettant de traiter un fil de matière rétrécissable qui comprend les étapes:
- de passage du fil (1) à une première vitesse, dans une ouverture d'entrée (17) à une extrémité d'une section (18) en forme d'entonnoir et formant les plis, munie de parois convergentes (19) qui définissent une ouverture de dégagement à l'autre extrémité de la section, ladite ouverture d'entrée (17) étant plus grande que l'ouverture de dégagement (20);
- de passage du fil replié par une ouverture resserrée d'entrée dans une chambre définie par des parois et comportant plusieurs sections comprenant une section de raccord (23) et les première (24) et seconde (25) sections de traitement à la vapeur, ladite chambre étant reliée à l'ouverture de dégagement de la section (18) formant les plis, et ladite ouverture d'entrée de la chambre étant plus petite que l'ouverture d'entrée (17) de la section (18) formant les plis, cette chambre comprenant en outre une ouverture de sortie du fil,
où l'action duale des parois convergentes de la section formant les plis et du fil qui traverse ladite ouverture d'entrée limitée de la chambre forme plusieurs plis dans le fil,
où la vapeur est introduite dans la seconde section de traitement (25) à la vapeur, qui se situe entre les ouvertures d'entrée et de sortie de la chambre, cette vapeur entrant:
dans un sens, dans la seconde section de traitement (25) à la vapeur, après quoi elle traverse cette section et entre dans la première section de traitement (24) à la vapeur et, de là, entre dans la section de raccord (23) puis se dirige vers l'ouverture d'entrée (17) de la section formant les plis et
dans l'autre sens, dans la seconde section de traitement (25) à la vapeur, qu'elle traverse, après quoi elle se dirige vers l'ouverture de sortie (26) de la chambre,
- d'engagement des plis du fil au fur et à mesure de son entraînement dans la section formant les plis et dans l'ouverture d'entrée (17) de la chambre, avec des ergots (27) disposés sur une chaîne sans fin (28) entraînée à une seconde vitesse inférieure à la première vitesse
- d'entraînement du fil replié dans la section de raccord (23) à ladite seconde vitesse et
les plis du fil étant tous en contact avec les parois de la chambre définissant la section de raccord (23) pendant une partie substantielle de leur passage dans cette section, ce qui permet de pratiquement éliminer la perte de vapeur par l'ouverture d'entrée de la section formant les plis (18),
la vapeur passant dans cette section de raccord faisant rétrécir le fil, de sorte que la superficie de sa section est plus petite que sa superficie lors de son entrée dans cette section
- de passage du fil replié par une ouverture resserrée d'entrée de la première section de traitement, ladite ouverture d'entrée étant plus petite que l'ouverture resserrée d'entrée de la chambre
- de passage du fil par la première section de traitement (24) à ladite seconde vitesse, les plis du fil, rétrécis dans la section de raccord (23), étant essentiellement en contact avec les parois définissant la première section de traitement (24) pendant une grande partie de leur déplacement dans cette section, ce qui permet en outre d'éviter que toute vapeur passant par cette section et par la section de raccord (23) s'échappe par l'ouverture d'entrée de la section formant les plis.

10. Procédé selon la revendication 9, dans lequel la chaîne engage deux fils, un de chaque côté, et leur fait traverser la chambre à ladite seconde vitesse.

11. Procédé selon la revendication 9 ou la revendication 10, dans lequel l'ouverture resserrée d'entrée de la chambre est reliée à l'ouverture de dégagement de la section formant les plis (18) par une surface conique.

12. Procédé selon l'une des revendications 9, 10 ou 11, dans lequel l'ouverture resserrée d'entrée de la première section de traitement (24) est reliée à la section de raccord (23) par une surface conique.

13. Appareil permettant de traiter un fil de matière rétrécissable qui comprend:
un moyen permettant de faire passer le fil (1) à une première vitesse par une ouverture d'entrée (17) à une extrémité d'une section en forme d'entonnoir et formant les plis (18), ladite section étant munie de parois convergentes (19) qui définissent une ouverture de dégagement à l'autre extrémité de la section et ladite ouverture d'entrée (17) étant plus grande que l'ouverture de dégagement (20);
un moyen permettant de faire passer le fil replié par une ouverture d'entrée limitée d'une chambre définie par des parois et comportant plusieurs sections, dont une section de raccord (23) et des première (24) et seconde (25) sections de traitement à la vapeur, ladite chambre étant reliée à l'ouverture de dégagement de la section formant les plis (18), et ladite ouverture d'entrée de la chambre étant plus petite que l'ouverture d'entrée (17) de la section formant les plis (18), cette chambre étant en outre munie d'une ouverture de sortie du fil;
un moyen permettant d'introduire la vapeur dans la seconde section de traitement (25) à la vapeur, qui se situe entre les ouvertures d'entrée et de sortie de la chambre, de sorte que cette vapeur passe, dans un sens, dans la seconde section de traitement (25) à la vapeur, après quoi elle traverse cette section et entre dans la première section de traitement (24) à la vapeur et, de là, entre dans la section de raccord (23) puis se dirige vers l'ouverture d'entrée (17) de la section formant les plis et, dans l'autre sens, dans la seconde section de traitement (25) à la vapeur, qu'elle traverse, après quoi elle se dirige vers l'ouverture de sortie (26) de la chambre;
un moyen permettant d'engager les plis du fil au fur et à mesure de son entraînement dans la section formant les plis et dans l'ouverture d'entrée (17) de la chambre, avec des ergots (27) disposés sur une chaîne sans fin (28) entraînée à une seconde vitesse inférieure à la première vitesse;
un moyen permettant d'entraîner le fil replié dans la section de raccord (23) à ladite seconde vitesse, de sorte que les plis du fil soient essentiellement en contact avec les parois de la chambre définissant la section de raccord (23) pendant une partie substantielle de leur passage dans cette section, et que la vapeur passant dans cette section de raccord fasse rétrécir le fil afin que la superficie de sa section soit plus petite que sa superficie lors de son entrée dans cette section;
un moyen permettant de faire passer le fil replié par une ouverture d'entrée limitée de la première section de traitement, ladite ouverture d'entrée étant plus petite que l'ouverture resserrée d'entrée de la chambre; et
un moyen permettant de faire passer le fil par la première section de traitement (24) à ladite seconde vitesse, de sorte que les plis du fil, rétrécis dans la section de raccord (23), soient essentiellement en contact avec les parois définissant la première section de traitement (24) pendant une grande partie de leur passage dans cette section.
